

1

3,052,571

### METHOD OF WATERPROOFING LEATHER

Charles A. Fetscher, Short Hills, and Stanley Lipowski, Newark, N.J., assignors to Nopco Chemical Company, Harrison, N.J., a corporation of New Jersey  
No Drawing. Filed July 11, 1958, Ser. No. 747,818

9 Claims. (Cl. 117—142)

This invention relates to a new and improved process for the waterproofing of leather. More particularly, the invention relates to a waterproofing process which is especially well suited for use in connection with the waterproofing of white leathers.

For obvious reasons, waterproofing is an extremely important step in the finishing of leather. However, it is of equal importance that the waterproofing of leather be accomplished without adversely affecting the air permeability or water-vapor permeability of the leather and without discoloring or darkening the leather. Many methods have been disclosed in the prior art as being suitable for use in rendering leather waterproof. Some of these have been more satisfactory than others. In most cases the proposed methods have been successful in providing the leather with the desired resistance to penetration by water or moisture. In many instances, however, this has been accomplished only by sacrificing the permeability of the leather to air and water-vapor. In other instances, the desired waterproofing has been achieved but with a discoloring or darkening of the leather.

In all probability the most well known of the prior art leather waterproofing processes involves the drumming of emulsions of a wax or grease into the tanned skin prior to drying same. More recently, improved methods for the waterproofing of leather have been devised. These involve, for example, the treatment of leather with oil-in-water emulsions of various water-insoluble organic polymers.

In addition to the aforementioned methods, other waterproofing processes have been disclosed in the art. Thus, for example, it is well known that penetration of waterproofing compounds into leather is facilitated when such compounds are added to the leather in the form of an organic solvent solution thereof. When such solutions are used, the waterproofing compounds appear to coat the surface of the fibers. The provision of such a coating is to be contrasted with the result obtained by certain of the previous mentioned methods wherein the waterproofing agent appears merely to be deposited in the spaces between the fibers.

A flow sheet representing in a schematic fashion the process of the invention is as follows:



2

The object of this invention is to provide a new and improved process for the waterproofing of leather.

A more particular object of the invention is to provide a method whereby leather is rendered waterproof without darkening or discoloring same or without adversely affecting the water-vapor or air permeability thereof.

Other objects of the invention will be obvious and they will in part appear hereinafter.

It has been discovered that the objects of this invention can be accomplished by treating leather which has been saturated thoroughly with an organic solvent solution of aluminum isopropoxide with an organic solvent solution of a soap-forming acid and subsequently washing and drying same.

The present invention contemplates the use and the treatment of tanned leather in air-dried condition. Preferably, our waterproofing process is carried out on the air-dried leather immediately after the fat-liquoring step. If desired, however, leather can be waterproofed by our method either prior to the fat-liquoring step or at any finishing step subsequent to fat-liquoring.

Furthermore, the process of the invention is such that it can be utilized in the treatment of leathers, without regard to the manner in which the leather has been tanned. Thus, for example, the invention can be practiced on leathers which have been subjected to chrome tannage, alum tannage, vegetable tannage, zirconium tannage and synthetic tannages, as well as on leathers which have been retanned.

The process of the invention can be adapted readily for commercial use. This will be readily apparent from the description which follows hereinafter. In carrying out the process, a dilute organic solvent solution of aluminum isopropoxide is first prepared. In general, any organic solvent in which aluminum isopropoxide is soluble can be used in the preparation of this solution. In the preferred embodiment of the invention, however, aromatic hydrocarbon solvents, such as, benzene, toluene, xylene, etc. are employed. The concentration of the solution used may be varied over a relatively wide range. Preferably, a solution containing from about 3.0% to about 10.0% by weight of aluminum isopropoxide will be employed. It should be understood, however, that more dilute or more concentrated solutions can be employed in carrying out the process, if desired. However, it has been our experience, that by far the most satisfactory results are obtained when a solution containing not less than 3.0%, by weight, or more than 10.0%, by weight, of aluminum isopropoxide is used.

In the first step of the preferred procedure, the tanned leather is thoroughly impregnated or saturated with the organic solvent solution of aluminum isopropoxide thus prepared. In general, this can be accomplished in any convenient manner. For all practical purposes, however, the complete saturation of the leather with the solution can be brought about most efficiently by totally immersing the leather in the solution in a suitable vessel containing the solution, as, for example, in a drum or vat.

The step of saturating the leather with the solvent solution of aluminum isopropoxide can be, and is preferably, carried out at a temperature which is at or near ordinary room temperatures. However, the solvent solution can be heated to a temperature which is elevated somewhat above room temperatures, if desired, prior to impregnating it into the leather which is to be waterproofed. It has been found that the use of a heated solvent solution during the step will facilitate, to some extent, the penetration of the aluminum isopropoxide solution into the leather. This means that, in such instances, complete saturation of the leather with the solution can be accomplished in a shorter period of time. However, since even at room temperatures adequate sat-

ration can be achieved by immersing the leather in a solution for as short a period as fifteen minutes, from an economical standpoint there is no real advantage in using a heated solvent solution. In any event, seldom, however, will it serve any useful purpose to immerse the leather in a solution which has been heated to a temperature above about 50° C.

The exact volume of the aluminum isopropoxide solution which is employed in the practice of our invention is not particularly critical. When the aluminum isopropoxide is introduced into the leather by an immersion process, the bath used, however, should contain a quantity of aluminum isopropoxide which is sufficient to impregnate all of the interstices of the leather. Obviously, volume of the solution which must be used in any particular instance will depend, at least in part, on the concentration of the solution. A lesser volume of a more highly concentrated solution and a greater volume of a more dilute solution will be needed to supply a sufficient quantity of impregnant. As a general rule, it has been found that the use of a solution containing from 3.0% to 10.0% by weight of aluminum isopropoxide, in a sufficiently large volume to permit the complete immersion therein of the leather to be waterproofed, will insure the presence of a quantity of aluminum isopropoxide which is more than enough for our purposes. It may be noted in this regard that the use of a solution containing a greater quantity of aluminum isopropoxide than is actually necessary does not render the process economically disadvantageous. After the saturated leather has been withdrawn from the bath, one can determine, by analytical methods, the quantity of aluminum propoxide remaining in the bath. The unused aluminum isopropoxide solution can be used over and over again in subsequent runs, preferably after it has been replenished by the addition of a quantity of aluminum isopropoxide sufficient to restore it to its original concentration.

In the second step of the preferred procedure, the aluminum isopropoxide-saturated leather is treated with an organic solvent solution of a soap-forming fatty acid. This can be accomplished in any convenient manner but preferably the step is carried out by immersing the saturated leather in a solution of the fatty acid. The treatment of the saturated leather with the solvent solution of fatty acid results in the formation, in situ, of the waterproofing aluminum salt of the fatty acid within the interstices of the leather. Isopropyl alcohol is also formed. The formation of the water-insoluble aluminum salt in this unique manner greatly enhances the resistance of leather to penetration by water and moisture. In the next step, the final step of the process, the leather is washed free of any unreacted aluminum isopropoxide and fatty acid present by means of the use of a suitable organic solvent. After washing, the waterproofed leather is permitted to dry at room temperature.

As indicated heretofore, the second step of the process contemplates the use of a solution of, what has been referred to as, a soap-forming fatty acid. By this we mean that a solution of an aliphatic monocarboxylic acid, either saturated, unsaturated or hydroxylated, which has a carbon chain length of from about 12 to about 24 carbon atoms is employed. Thus, for example, solutions of soap-forming fatty acids, such as lauric acid, myristic acid, palmitic acid, stearic acid, behenic acid, oleic acid, ricinoleic acid, etc., or mixtures of one or more of these, are fully suited for use. In the preferred embodiment of the invention a solution of lauric acid, oleic acid or stearic acid is employed.

Any organic solvent in which the fatty acid is soluble and which, at the same time, is miscible with the solvent used in the preceding step of the process can be used both in producing the fatty acid solution employed in the second step and in the washing operation of the third step. In the preferred practice of the invention, however, aromatic hydrocarbon solvents, such as, benzene, toluene,

xylene, etc., are used both in the second and third steps. In the second step, solutions containing from about 3.0% to 10.0% by weight of the soap-forming fatty acid are preferably employed. However, more dilute or more concentrated solutions can be used, if desired. No particular advantage is gained, however, by the use of a solution which contains less than 3.0% by weight or more than 10.0% by weight of the soap-forming fatty acid.

The precise volume of the fatty acid solution used in the practice of the invention is not particularly critical. For maximum effectiveness, however, a sufficient quantity of fatty acid must be provided to react with all of the aluminum isopropoxide present in the interstices of the leather. The use of a solvent solution containing from about 3.0% to 10.0% by weight of fatty acid in a sufficiently large volume to permit the complete immersion therein of the leather to be treated will provide the system with a quantity of fatty acid which is more than enough for our purposes. The use, or presence, of an excess of acids in the bath is not economically disadvantageous since the bath can be used over and over again in subsequent runs, preferably after it has been replenished by the addition of a quantity of fatty acid sufficient to return it to its original concentration.

The treatment of the aluminum isopropoxide-saturated leather with the solution of the soap-forming fatty acid can be, and is preferably, carried out at temperatures which are at or near ordinary room temperatures. Solvent solutions of the fatty acid heated to temperatures of up to about 50° C. can be used, however, if desired. It has been observed that, when a heated solution of fatty acid is used, the rate of the reaction of the fatty acid with the aluminum isopropoxide is accelerated to some extent. Thus, for example, using an unheated solvent solution, the reaction will proceed to substantial completion when the saturated leather is allowed to stand in contact with the fatty acid solution for a period of about fifteen minutes. A ten minute immersion period will, on the other hand, often be sufficient when the fatty acid solution is pre-heated to about 50° C. Since, for all practical purposes this difference is not deemed to be too highly significant, the reaction is preferably allowed to occur at ordinary room temperatures.

As indicated heretofore, the third step in our process involves washing the treated leather in a solvent, such as, an aromatic hydrocarbon, to remove any unreacted ingredients present. This step is carried out at room temperature preferably but, as was the case with the preceding steps in the process, it too can be carried out at elevated temperatures, that is, temperatures up to about 50° C., if desired. The washing operation can be performed in any convenient manner but it is most easily accomplished by immersing the treated leather in a vat or drum of fresh solvent. Alternate methods for accomplishing the desired result, however, will be readily apparent to persons skilled in the art. Immersion of the treated leather in the solvent for not longer than about ten minutes, and generally for about five minutes, will be sufficient washing in most instances.

Finally, when the washing step is completed, the leather is permitted to air dry. The waterproofed leather may be subjected thereafter to other conventional processing or finishing steps.

It should be understood that the sequence, disclosed heretofore, of treating the leather first with the aluminum isopropoxide solution and then with the fatty acid solution represents only the preferred method for practicing our invention. This sequence is not critical insofar as the operability of the invention is concerned and the order of the steps could be reversed, if desired. Thus, for example, the leather to be waterproofed could be saturated with the solvent solution of the fatty acid in the first step of the process and in the second step the saturated leather could be treated with the solvent

solution of the aluminum isopropoxide. The various disclosures heretofore with respect to the practice of the invention by preferred method are applicable equally with respect to the practice of the invention by the alternate procedure. As in the preferred method, treatment by the alternate procedure results in the impregnation of the interstices of the leather with the desired waterproofing aluminum salt.

Many advantages accrue from the practice of our invention. First, by its leathers which are highly resistant to penetration by water and moisture are obtained. Moreover, the process is economical and commercially feasible. It does not require the use of equipment not already in use in leather tanneries, and its practice does not necessitate a knowledge of special techniques. Furthermore, leather treated as disclosed herein is protected indefinitely. This is in contrast to leather which, in the prior art, has been surface treated with fats, waxes and preformed aluminum soaps. Such treatment affords temporary protection only. When the aluminum soap is formed in situ, by the two stage process described herein, it impregnates the leather. Permanent protection is thus provided since the impregnant cannot be abraded or washed away. Moreover, the process is noteworthy in that neither the air permeability nor the water-vapor permeability of the leather is adversely affected thereby. Finally, treatment by our process does not result in the discoloration or darkening of the leather. The latter feature will render the process invaluable for use in the waterproofing of light, and particularly white, leathers.

For a fuller understanding of the nature and objects of this invention, reference may be had to the following examples which are given merely as further illustrations of the invention and are not to be construed in a limiting sense. All parts given in the examples are parts by weight unless otherwise indicated.

*Example I*

Samples of side leather were waterproofed by process of the invention. The leather employed was chrome tanned, syntan retanned and fat-liquored.

A solution comprising benzene having dissolved therein 3.0% by weight of aluminum isopropoxide was first prepared. This solution was divided into two parts. A sample of side leather designated, hereinafter as sample I, was immersed in one of the parts of the solution. It was retained therein for a period of about 30 minutes. The solution had a temperature of about 27° C. Another sample of the same side leather, designated hereinafter as sample II, was immersed in the second part of the solution and retained therein for a period of about 15 minutes. The solution used had a temperature of about 27° C.

Each sample of leather was removed from the solution at the end of the designated time. Sample I was immediately immersed in a solution comprising 3.0% by weight of oleic acid in benzene and it was retained therein for a period of about 30 minutes. This solution had a temperature of about 27° C. Sample II was immediately immersed in a 3.0% by weight solution of oleic acid in benzene and retained therein for a period of about 15 minutes. This solution had a temperature of about 27° C.

At the end of the designated period of time, each of the samples of leather were removed from the oleic acid solution. Each was thereafter washed free of unreacted materials by immersion in benzene for a period of about 5 minutes. Each sample was thereafter removed and allowed to dry at room temperature. Each of the dry samples were tested for static water absorption by the American Leather Chemists Association Provisional Method, April 1953 (Test Method E 30). Static water absorption is defined therein as the amount of water absorbed by leather which is immersed without flexing in water for a specified period of time. The test method

contemplates two immersion periods in water, namely, 30 minutes and 120 minutes. The method gives an adequate indication of the percent of water absorbed by leather in the specified periods of time. The following are the results of the static water absorption tests.

|    | Immersion Period..... | Percent Water Absorption |             |
|----|-----------------------|--------------------------|-------------|
|    |                       | 30 minutes               | 120 minutes |
| 10 | Sample I.....         | 21.5                     | 31.8        |
|    | Sample II.....        | 24.3                     | 35.7        |

15 The foregoing procedure was repeated in every detail except that where a 3.0% by weight aluminum isopropoxide solution was employed originally, a 5.0% by weight solution thereof was instead used, and where 3.0% by weight of oleic acid solution was originally used, a 5.0% by weight of the oleic acid solution was instead employed. The samples of leather thus treated were tested for static water absorption in the same manner as were samples I and II. In the table which follows herein-after, the designation sample III refers to the product corresponding to previous sample I. The designation sample IV refers to the product corresponding to the previously mentioned sample II. The result of the static water absorption test were as follows:

|    | Immersion Period..... | Percent Water Absorption |             |
|----|-----------------------|--------------------------|-------------|
|    |                       | 30 minutes               | 120 minutes |
| 30 | Sample III.....       | 19.3                     | 28.2        |
|    | Sample IV.....        | 24.3                     | 32.2        |

35 The foregoing procedures were repeated in every detail once again except that, in this instance, 10.0% by weight solutions of aluminum isopropoxide in benzene and 10.0% by weight solutions of oleic acid in benzene were used instead of the 3.0% by weight and 5.0% by weight solutions previously employed. These samples were tested for static water absorption in the same manner as were samples I to IV, inclusive. In the table which follows herein-after, the designation sample V refers to a product corresponding to previously mentioned samples I and III. The designation, sample VI refers to a product corresponding to the previous samples II and IV. The results of these tests were as follows:

|    | Immersion Period..... | Percent Water Absorption |             |
|----|-----------------------|--------------------------|-------------|
|    |                       | 30 minutes               | 120 minutes |
| 50 | Sample V.....         | 24.7                     | 40.0        |
|    | Sample VI.....        | 19.7                     | 30.0        |

55 The foregoing results furnish conclusive evidence that excellent waterproofing can be achieved when leather is treated by the process of our invention. However, in order to demonstrate that the result obtained is attributable to a reaction between the aluminum isopropoxide and oleic acid, in situ, rather than merely to the deposition of a coating of water-insoluble fatty acid in or on the leather, the following experiments were carried out. A solution of 3.0% by weight of oleic acid dissolved in benzene and a solution of 5.0% by weight of oleic acid dissolved in benzene was first prepared. Into each of 60 the two solutions a sample of chrome tanned, syntan retanned and fat-liquored side leather was immersed. In one case, the leather was allowed to stand in contact with the 3% oleic acid solution for 30 minutes. The leather thus treated will be referred to herein-after as sample VII. 65 The second sample of leather herein-after, designated as

sample VIII, was allowed to stand in the 5% oleic acid solution for 30 minutes.

At the end of the designated immersion periods each sample of leather was removed from the oleic acid solution and air-dried. They were then tested for static water absorption in the same manner as were samples I through VI inclusive. The results of these tests were as follows:

| Immersion Period | Percent Water Absorption<br>(Samples Treated With Fatty Acid Only) |             |
|------------------|--------------------------------------------------------------------|-------------|
|                  | 30 minutes                                                         | 120 minutes |
| Sample VII       | 116<br>95                                                          | 116<br>97   |
| Sample VIII      |                                                                    |             |

Since it is well known in the art that the properties of aluminum isopropoxide are such, that it alone could not be used and would not function as a waterproofing agent and since the foregoing results demonstrate that oleic acid alone is ineffective, the results of the static water absorption tests reported herein conclusively prove that the present process provides a valuable method of waterproofing leather.

An examination of the leather after treatment by the method disclosed herein reveals that in each instance the sample was waterproofed without sacrificing the air and water vapor permeability thereof and without darkening or discoloring the leather.

#### Example II

In this example the procedure of Example I was repeated in every detail except that calfskin rather than side leather was employed in this example. The calfskin used was chrome tanned and syntan retanned but it had not been fat-liquored prior to waterproofing.

Calfskin (sample I) was treated at a temperature of 27° C. by immersing it first in a 3.0% by weight solution of aluminum isopropoxide in benzene for 30 minutes and thereafter in a 3.0% by weight solution of oleic acid in benzene for 30 minutes. The leather was then washed in benzene for 5 minutes and finally air-dried.

Calfskin (sample II) was treated at a temperature of 27° C. by immersing it first in a 5.0% by weight solution of aluminum isopropoxide in benzene for 30 minutes and thereafter in a 5.0% by weight solution of oleic acid in benzene for 30 minutes. The leather sample was then washed in benzene for a period of about 5 minutes and finally air-dried.

Calfskin (sample III) was treated at a temperature of about 27° C. by immersing it first in a 10.0% by weight solution of aluminum isopropoxide in benzene for 30 minutes and thereafter in a 10.0% by weight solution of oleic acid in benzene for 30 minutes. The leather sample was then washed in benzene for about 5 minutes and finally air-dried.

Calfskin (sample IV) was treated in the same manner as sample I except that it was immersed in the benzene solutions of aluminum isopropoxide and oleic acid for 15 minutes rather than 30 minutes.

Calfskin (sample V) was treated in the same manner as sample II except that it was immersed in the benzene solutions of aluminum isopropoxide and oleic acid for 15 minutes each rather than 30 minutes.

Calfskin (sample VI) was treated in the same manner as sample III except that it was immersed in the benzene solutions of aluminum isopropoxide and oleic acid for 15 minutes each rather than 30 minutes.

Calfskin (sample VII) was treated in the same manner as sample I except that the benzene solutions of aluminum isopropoxide and oleic acid were heated to a temperature of 50° C. prior to immersing the leather therein and except that the leather was allowed to remain immersed in each of the solutions for 10 minutes rather than for 30 minutes.

Calfskin (sample VIII) was treated in the same manner as sample II except that the solutions of aluminum isopropoxide and oleic acid used were heated to a temperature of 50° C. prior to immersing the leather therein and except that the leather was allowed to remain immersed in each solution for 10 minutes rather than 30 minutes.

Calfskin (sample IX) was treated in the same manner as sample III except that the solutions of aluminum isopropoxide and oleic acid were heated to a temperature of 50° C. prior to immersing the leather therein and except that the leather was allowed to remain immersed in each solution for 10 minutes rather than 30 minutes.

For comparative purposes the basic procedure employed in treating each of samples I to III, inclusive, and VII through XI, inclusive, of this example was repeated in every detail except that the steps of immersing the leather in the solution of aluminum isopropoxide and the step of finally washing the treated leather in benzene were omitted. In the tables which follow hereinafter the samples corresponding to samples I, II, III, VII, VIII and IX are designated as samples X, XI, XII, XIII, XIV and XV respectively.

Each of the dry samples were tested for static water absorption by the Provisional Method of the American Leather Chemists Association, April 1953, referred to heretofore. The following are the results of those tests:

| 30               | Percent Water Absorption |             |
|------------------|--------------------------|-------------|
|                  | 30 minutes               | 120 minutes |
| Immersion Period |                          |             |
| Sample I         | 18.2                     | 27.6        |
| Sample II        | 17.4                     | 26.3        |
| Sample III       | 8.0                      | 16.2        |
| Sample IV        | 19.4                     | 29.0        |
| Sample V         | 17.2                     | 28.0        |
| Sample VI        | 13.9                     | 23.0        |
| Sample VII       | 16.8                     | 28.5        |
| Sample VIII      | 16.2                     | 27.8        |
| Sample IX        | 13.0                     | 24.4        |

| 40               | Percent Water Absorption |             |
|------------------|--------------------------|-------------|
|                  | 30 minutes               | 120 minutes |
| Immersion Period |                          |             |
| Sample X         | 110.5                    | 113         |
| Sample XI        | 107                      | 108         |
| Sample XII       | 115.5                    | 108         |
| Sample XIII      | 135                      | 138         |
| Sample XIV       | 137                      | 137         |
| Sample XV        | 142                      | 142         |

These results demonstrate the extent to which leather treated by our method was rendered water-repellant. It was further observed that this result was accomplished without darkening or discoloring and without adversely affecting the air or water permeability of the leather.

#### Example III

60 In this example, samples of chrome tanned side leather were treated.

A solution of 3.0% by weight of aluminum isopropoxide was first prepared. This was divided into three parts. A separate sample of leather was immersed in each solution and retained therein for a period of about 30 minutes.

65 The temperature of the solution used in each instance was about 27° C. At the end of the designated immersion period each sample of leather was removed from its aluminum isopropoxide bath. The first, sample I, was immediately immersed in a bath of 3.0% by weight oleic acid in benzene and retained therein for a period of about 30 minutes. The second, sample II, was immersed in a bath of 3.0% by weight of stearic acid in benzene and retained therein for about 30 minutes. The third, sample III, was immersed in a bath of 3.0% by weight lauric acid and re-

tained therein for 30 minutes. In each instance, the temperature of the fatty acid solution employed was 27° C. After 30 minutes each sample was removed from its fatty acid bath and washed free of unreacted materials by immersion in benzene for about 5 minutes. Each sample was removed thereafter and allowed to dry at room temperature.

For comparative purposes, the procedure used in waterproofing each of the samples I, II and III was repeated except that in each instance the steps of immersing the leather in the aluminum isopropoxide solution and of washing the leather in benzene were omitted. In the tables which follow hereinafter, the comparative samples which correspond to samples I, II and III have been designated at samples IV, V and VI respectively.

Each of these six samples of treated leather were tested for static water absorption by the Provisional Method of American Leather Chemists Association, April 1953, referred to in Example I. The results of the tests thus conducted were as follows:

| Immersion Period..... | Percent Water Absorption |             |
|-----------------------|--------------------------|-------------|
|                       | 30 minutes               | 120 minutes |
| Sample I.....         | 21.5                     | 31.8        |
| Sample II.....        | 17.6                     | 27.4        |
| Sample III.....       | 17.9                     | 27.9        |

  

| Immersion Period..... | Percent Water Absorption<br>(Samples Treated With Fatty Acid Only) |             |
|-----------------------|--------------------------------------------------------------------|-------------|
|                       | 30 minutes                                                         | 120 minutes |
| Sample IV.....        | 116                                                                | 116         |
| Sample V.....         | 85                                                                 | 90          |
| Sample VI.....        | 91                                                                 | 96          |

#### Example IV

In this example, chrome tanned, high grade sheepskin, a soft leather of the type used in the glove and garment industries, was employed. The leather was fat-liquored and air-dried prior to use.

A sample of this leather, hereinafter referred to as sample I, was immersed first in a solution of 3.0% by weight of aluminum isopropoxide in benzene and retained therein for 30 minutes. The solution used had a temperature of 27° C. After immersion in this solution, the leather sample was removed and it was immersed immediately in a solution of 3.0% by weight stearic acid in benzene and retained therein for a period of 30 minutes. The stearic acid solution used had a temperature of 27° C. At the end of the designated period of time the sample was removed from the stearic acid solution, immersed in benzene and retained therein for 5 minutes and thereafter air-dried.

The dynamic water resistance of the leather thus treated was tested by the American Leather Chemists Association Provisional Method, April 1953 (Test Method E 31). For comparative purposes, a sample of non-waterproofed sheepskin which was chrome tanned and fat-liquored was subjected to the same test method. This non-waterproofed leather sample will be referred to hereinafter as sample II. For further comparison, chrome tanned sheepskin, which after fat-liquoring and drying, was waterproofed using chromium couples was also subjected to the dynamic water resistance test. This sample will be referred to as sample III. Finally, chrome tanned sheepskin which, after fat-liquoring and drying, had been waterproofed using chromium couples and which was further subjected to the treatment given to sample I of this exam-

ple was also tested for dynamic water absorption. This is sample IV.

The test for dynamic water absorption revealed that, of all the samples tested, sample I, that is, leather treated by the process of this invention, was most resistant to the penetration of water. Initial water penetration of sample I occurred only after 7,500 cycles. The test proved sample IV to be second best, with water penetrating the leather only after 6,500 cycles, sample III was shown to be third best, with water penetrating the leather only after 5,500 cycles. In the case of sample II, water penetrated the leather almost instantly.

The American Leather Chemists Association Test for static water absorption was then carried out in connection with samples I and III. It was found that sample III which was waterproofed using only chromium couples took up as much as 107% water whereas sample I absorbed only 32% in the same period of time.

The foregoing results conclusively demonstrate that superior waterproofing of leather is provided by the process of the present invention. In addition, examination of leather which was subjected to the method disclosed herein revealed that the desired water repelling properties were achieved without darkening or discoloring of the leather.

Having described our invention what we claim as new and desire to secure by Letters Patent is:

1. A method of waterproofing leather with an aluminum salt of an aliphatic monocarboxylic acid having a carbon chain length of from about 12 to about 24 carbon atoms consisting essentially of impregnating tanned leather with a solution consisting of an aromatic hydrocarbon and aluminum isopropoxide, and with a solution consisting of an aromatic hydrocarbon and an aliphatic monocarboxylic acid having a carbon chain length of from about 12 to about 24 carbon atoms and subsequently washing the leather thus treated with an aromatic hydrocarbon solvent.

2. Tanned leather produced by the process of claim 1 characterized by its water repellency, the permanency of its water repellency, and its air permeability and water vapor permeability and further characterized in that it is not discolored or darkened as a result of that process.

3. A method of waterproofing leather with an aluminum salt of an aliphatic monocarboxylic acid having a carbon chain length of from about 12 to about 24 carbon atoms consisting essentially of immersing tanned leather in a solution consisting of an aromatic hydrocarbon and from about 3.0% to about 10.0% by weight of aluminum isopropoxide for a period of time sufficient to saturate said leather with said solution, immersing said leather in a solution consisting of an aromatic hydrocarbon and from about 3.0% to about 10.0% by weight of an aliphatic monocarboxylic acid having a carbon chain length of from about 12 to about 24 carbon atoms and subsequently washing the leather thus treated by immersing it in an aromatic hydrocarbon solvent.

4. A method of waterproofing leather with an aluminum salt of an aliphatic monocarboxylic acid having a carbon chain length of from about 12 to about 24 carbon atoms consisting essentially of immersing tanned leather in a solution consisting of an aromatic hydrocarbon and from about 3.0% to about 10.0% by weight of an aliphatic monocarboxylic acid having a carbon chain length of from about 12 to about 24 carbon atoms for a period of time sufficient to saturate said leather with said solution, immersing said leather in a solution consisting of an aromatic hydrocarbon and aluminum isopropoxide and subsequently washing the leather thus treated by immersing it in an aromatic hydrocarbon solvent.

5. A method of waterproofing leather with an aluminum salt of an aliphatic monocarboxylic acid having a carbon chain length of from about 12 to about 24 carbon atoms consisting essentially of immersing tanned leather in a solution consisting of about 3.0% to about 10.0% by weight of aluminum isopropoxide and an aromatic hydro-

carbon solvent selected from the group consisting of benzene, toluene and xylene for a period of time sufficient to saturate said leather with said solution, immersing said leather in a solution consisting of 3.0% to about 10.0% by weight of an aliphatic monocarboxylic acid having a carbon chain length of from about 12 to about 24 carbon atoms in an aromatic solvent selected from the group consisting of benzene, toluene and xylene and subsequently washing the leather thus treated by immersing it in an aromatic hydrocarbon solvent selected from the group consisting of benzene, toluene and xylene.

6. A method of water-proofing leather with an aluminum salt of a fatty acid selected from the group consisting of lauric acid, stearic acid and oleic acid consisting essentially of immersing tanned leather in a solution consisting of from about 3.0% to about 10.0% by weight of aluminum isopropoxide and the remainder being an aromatic hydrocarbon selected from the group consisting of benzene, toluene and xylene for a period of time sufficient to saturate said leather with said solution, immersing said leather in a solution consisting of from about 3.0% to about 10.0% by weight of an aliphatic monocarboxylic acid selected from the group consisting of lauric acid, stearic acid and oleic acid and the remainder being an

aromatic hydrocarbon selected from the group consisting of benzene, toluene and xylene and subsequently washing the leather thus treated by immersing it in an aromatic hydrocarbon selected from the group consisting of benzene, toluene and xylene.

5 7. The process of claim 6 wherein the aliphatic monocarboxylic acid employed is lauric acid.

8. The process of claim 6 wherein the aliphatic monocarboxylic acid employed is stearic acid.

10 9. The process of claim 6 wherein the aliphatic monocarboxylic acid employed is oleic acid.

References Cited in the file of this patent

UNITED STATES PATENTS

|    |           |             |       |               |
|----|-----------|-------------|-------|---------------|
| 15 | 1,242,327 | Cuthbertson | ----- | Oct. 9, 1917  |
|    | 2,182,045 | Bell        | ----- | Dec. 5, 1939  |
|    | 2,323,387 | Edelstein   | ----- | July 6, 1943  |
|    | 2,603,576 | Cook et al. | ----- | July 16, 1952 |
| 20 | 2,670,303 | Mailander   | ----- | Feb. 23, 1954 |

FOREIGN PATENTS

|         |               |       |                |
|---------|---------------|-------|----------------|
| 609,002 | Great Britain | ----- | Sept. 23, 1948 |
| 767,585 | Great Britain | ----- | Feb. 6, 1957   |